

## UNITED STATES PATENT OFFICE

2,326,842

## TREATMENT OF ARTIFICIAL MATERIALS

Henry Dreyfus, London, England, assignor to  
Celanese Corporation of America, a corpora-  
tion of Delaware

No Drawing. Application March 6, 1942, Serial  
No. 433,575. In Great Britain February 22,  
1939

11 Claims. (Cl. 8—132)

This invention relates to improvements in the treatment of artificial filaments and other products and is more particularly concerned with improving the tenacity and/or the extensibility of such materials.

This application is a continuation-in-part of my application S. No. 318,711, filed February 13, 1940.

It has been known for some time that the tenacity of materials made of organic derivatives of cellulose is increased by stretching the materials, the stretching being facilitated by so-called assisting agents which are solvents or strong swelling agents for the organic derivative of cellulose. A large number of such assisting agents has been proposed including both water-miscible and water-immiscible agents. In general the stretching is best carried out on the running filaments or other products which, after being gripped by a pair of nip rollers or other non-slip feed device, may be carried through a bath of the assisting agent and be taken up at the other end of the bath by a similar pair of rollers or other feed device rotating at a higher speed than the feed-in device. It is generally advantageous to arrange that the stretch takes place in stages by arranging a number of gripping devices along the bath, the various devices rotating at increasing speeds as the filaments proceed along the bath. However, the second set of gripping devices may rotate at the same speed as the feed-in set, so as not to impart a stretch during the preliminary soaking of the material.

As is well known, it is of great importance in textile-forming operations, e. g. weaving and knitting, that the yarns or other filamentary materials should possess a considerable extensibility so that they may be able to withstand the relatively violent tensioning and flexing to which they are subjected during those operations. In U. S. Patent No. 2,058,422, processes are described whereby the extensibility of materials made of organic derivatives of cellulose is increased by subjecting the materials, in the absence of tension sufficient to stretch them, to treatment with organic solvents, latent solvents or swelling agents. The treatment is of greatest value for improving the extensibility of filaments, yarns and the like of cellulose derivatives which have either during or subsequent to the spinning operation been subjected to a stretch for the purpose of improving the tenacity. Such an increased tenacity, for example a tenacity of 3 or 4 grams per denier or more, is usually accompanied by an undesirably low extensibility. Such materials

may, for example, be produced by stretching already formed, for example dry-spun, cellulose derivative filaments or yarns by the processes described above, e. g. by those of U. S. Patent

5 No. 2,047,195 and British Patents Nos. 323,790, 370,430 and 378,074 using organic solvents as the stretch-assisting agents, or by the processes of U. S. Patents Nos. 2,142,717 and 2,142,722 and British Patents Nos. 438,584, 538,585, 438,586, and 10 438,587 using steam or hot water under pressure as the stretch-assisting agent. Again, in the wet spinning processes of U. S. Patents Nos. 2,147,640, 2,179,544 and 2,086,122 and British Patents Nos. 177,868, 179,234, 340,326, 340,436 and 340,437 the 15 nature of the coagulating bath is such that the filaments may be drawn out to very fine deniers and as a consequence have a high tenacity. All these materials are considerably improved by applying the treatment of U. S. Patent No. 2,058,422 20 to increase their extensibility.

The present invention relates to a new method of applying water-insoluble organic solvents, latent solvents and other swelling agents which are to serve as stretch-assisting agents in operations whereby the tenacity of the treated materials may be increased or as shrinking agents in treatments whereby the treated materials may be given an improved power of withstanding textile-forming operations. According to the present invention these agents are applied to the materials, such as, for example, yarns and filaments, before they are subjected to a textile-forming operation, in the form of aqueous emulsions. By this means, the tendency of the constituents of 25 the bath, particularly highly volatile constituents, to evaporate is considerably reduced, and in consequence it is much easier to maintain the composition of the bath constant. Moreover, when employing the aqueous emulsions according to the invention there is no need to dry the materials out before they are treated with the emulsions and further the possible shrinkage which the materials undergo may be readily controlled.

45 The emulsions may be made up in any desired manner and are usually best prepared with the aid of emulsifying agents, for example soaps, e. g. alkali metal and ammonium soaps, and ethanolamine and other organic soaps, particularly 50 soaps of saturated higher fatty acids, sulphonated fatty alcohols, the alkylated naphthalene sulphonic acids, and particularly the higher alkylated naphthalene sulphonic acids, such as cetyl naphthalene sulphonic acid, and the Twitchell type of fat splitting agent obtained, for ex-

ample, by the sulphonation of a mixture of naphthalene and castor oil. If desired, the emulsions may be stabilised with the aid of suitable protective colloids, e. g. a water-soluble methyl cellulose.

The most important class of swelling agents for use according to the present invention comprises the latent solvents, particularly the chlorinated hydrocarbons, e. g. methylene chloride, ethylene chloride and chloroform. The disperse phase in the emulsion may consist of 100% of the latent solvent or other water-insoluble swelling agent for the cellulose derivative, or the swelling agent may be suitably diluted in the disperse phase with water-insoluble diluents, for example benzene, toluene, xylene and other cyclic hydrocarbons, benzine, petrol ether, kerosene and other hydrocarbons of the aliphatic series, carbon tetrachloride, trichlorethylene, perchlorethylene and other chlorinated or halogenated compounds which are inert or comparatively inert towards the cellulose derivatives. Preferably the swelling agent constitutes at least about 50% by volume of the disperse phase. For example, a very suitable disperse phase for the treatment of ordinary acetone-soluble cellulose acetate materials consists of a solution of methylene chloride in benzene, high-boiling petroleum or carbon tetrachloride having a concentration of the order of 50-80% by volume. The concentration of the disperse phase in the emulsion may be set at any desired value. The lower concentrations of the disperse phase are more suitable where hanks are being treated and where the time of treatment is comparatively long. However, with a view to uniformity of treatment it is undesirable to employ concentrations of the disperse phase of much under 10% by volume, and for the treatment of travelling materials it is preferable that the concentration should be considerably higher, for example over 20%, especially 30-50 or 55% by volume.

The temperature of treatment depends upon the degree of modification of characteristics which is desired, upon the nature of the materials treated, and upon the nature and concentrations of the treatment medium. In general, however, a temperature of the order of 15-30° C., e. g. 25° C., is preferable. The treatment may be carried out under super-atmospheric pressure, if desired, with a view to accelerating the action of the medium, though, in general it is preferable to treat hanks of material under normal pressure, in which case a time of treatment of 10 minutes is usually found sufficient to produce substantially the maximum increase in extensibility for the particular medium or to give substantially the maximum degree of stretch assistance. The time of treatment may, however, be extended up to one or two hours or more, if desired. When treating travelling materials, the medium may be allowed to act while the materials are passing through a pressure chamber.

Treatments according to the invention may be applied to the materials in any suitable form. Thus, when it is desired to stretch them, hanks may be immersed in the emulsion, the hanks being supported, for example, on rollers, the distance apart of which may be increased, and when it is desired to shrink them, hanks may be suspended in the emulsions from rods or other devices common in the dyeing industry. Again the materials may be caused to travel through the treatment liquor by means of rollers suit-

ably disposed in the liquor or above the liquor, in the latter case suitable guides being provided to immerse the filaments or yarns. Alternatively, the materials in hank form or travelling materials may be sprayed with the emulsions. A treatment of travelling materials is particularly convenient when it is desired to stretch the materials. A very convenient arrangement for the treatment of travelling materials is to carry the materials successively round a number of sets of rollers, each set consisting of three rollers arranged at the apices of a triangle. The base of the triangle may be uppermost and the two rollers forming the base may be above the liquor, the remaining roller being in the liquor, or if desired this arrangement may be inverted, or alternatively the whole of the set of rollers may be out of the liquor and may be irrigated or sprayed with the emulsion of the solvent or swelling agent. Again, the materials may pass in contact with the upper surface of one or more rollers which dip into a bath of emulsion so as to carry a film of liquor from which the materials take up an appropriate amount. Even where some of the rollers of each set dip into the liquor it is desirable to irrigate or spray the rollers which are out of the liquor. The rollers may be arranged so that each set runs at a regulated higher or lower speed than the preceding set so as to stretch the materials or to enable shrinkage to take place. As already indicated, in some cases when it is desired to stretch the materials, particularly with assisting agents having a comparatively low penetrative power, it is desirable that the second set of rollers should run at the same speed or even a slightly reduced speed as compared with the first set, so as to enable the materials to be thoroughly soaked.

In order to avoid the delustering action of hot aqueous media on cellulose derivative materials in the presence of organic swelling agents, washing of the materials with aqueous media should be carried out at temperatures which do not exceed about 60° C., and preferably at temperatures of the order of 15-30° C. Removal of the organic swelling agents should accordingly precede any treatments with hot aqueous media to which it may be desired to subject the materials. The materials are preferably freed from the organic swelling agent by washing with an aqueous solution of an emulsifying agent, especially an aqueous solution of any emulsifying agent present in the treatment medium, followed by a water wash. However, other methods of removing the medium may be employed, e. g. a simple washing with water, particularly where uniformity of appearance in the products is of subsidiary importance.

The present invention enables the materials to be stretched within very wide limits; for instance comparatively small stretches may be imparted, e. g. of the order of 20-100% of the original length of the materials, or very much larger stretches such as 500-1000% or even several thousand per cent of the original length.

The stretched materials have an increased tenacity as compared with the starting materials. In some cases it is, however, desirable to subject them to a further process with the object of improving their extensibility. With this object in view they may be treated with agents which have a tendency to shrink the materials. Shrinking is not absolutely necessary, though it is desirable, and in this connection general reference is made to U. S. Patent No. 2,058,422 which has

this general object. As indicated in that specification, shrinkage of the order of 5-15% on the stretched length of the materials gives a very satisfactory increase in the extensibility of the stretched materials. Again, as indicated in that specification, the shrinking may take place continuously with the stretching operation, and indeed with the same agents as those used for stretching. Such agents may again be used in emulsified form as described above. In such a case the materials may be stretched by means of sets of rollers as described above, and then carried on to further sets of rollers driven at such speeds as to promote shrinkage of the materials, all the rollers being irrigated and/or sprayed with the emulsion of the agent used both to facilitate stretching and to bring about shrinkage.

It is to be understood that improvement in the materials can be effected even where the filaments or yarns are neither stretched nor shrunk, i. e. where they are held against shrinkage under a tension insufficient to stretch them. However, the best increase in extensibility is obtained when actual shrinkage takes place, for example a shrinkage of the order of 5-15% on the initial length of the materials under treatment, this being particularly the case with materials which have been stretched and which have a tenacity exceeding 2 grams per denier.

Acetone-soluble cellulose acetate has been mentioned in the preceding description, and this is the most important cellulose derivative. However, the invention is also applicable to the treatment of filaments, yarns and the like of other cellulose derivatives, for example cellulose formate, propionate, butyrate, nitro-acetate, acetate-propionate and acetate-butyrate and ethyl and benzyl celluloses, as well as cellulose ether-esters and mixed ethers. Further, in addition to the treatment of filaments, yarns and the like, the invention is also of importance for improving the properties of ribbons, strips and like materials made of the cellulose derivatives.

The following examples illustrate the invention:

*Example 1*

A cellulose acetate yarn having a low extensibility, produced by stretching the yarn to 1000% of its original length in wet steam, is immersed at 25° C. in hank form in a medium comprising a mixture of 55 parts of methylene chloride and 45 parts of high boiling petroleum dispersed in 100 parts of water (all parts by volume) with the aid of 1% by weight of ammonium stearate. After 10 minutes the yarn is withdrawn from the medium, washed at 25° C. first with a 1% solution of ammonium stearate in water and then with water, and finally dried in a stream of air. It is found to be well shrunk and to show a high extensibility.

*Example 2*

Dry-spun cellulose acetate yarn is withdrawn from bobbins and led to a series of rollers adapted to stretch it in eight stages by 250% of its original length. Before reaching the first of such rollers the yarn is passed through a bath of an emulsion comprising a mixture of 75 parts of methylene chloride and 25 parts of high boiling petroleum dispersed in 100 parts of water (all parts by volume) with the aid of 1% ammonium palmitate and the same medium is sprayed on to the travelling yarn between each stage of stretching. The yarn is then passed

over three rollers irrigated with a 1% ammonium palmitate solution in water and through a bath of water, and is finally dried in a stream of air. All the liquid media are maintained at 25° C.

*Example 3*

The yarn produced according to Example 2 is treated by the process of Example 1 and then found to possess a good tenacity and extensibility.

Having described my invention, what I desire to secure by Letters Patent is:

1. Process for increasing the extensibility of artificial filaments, threads, yarns and like materials containing organic derivatives of cellulose, which comprises subjecting stretched materials, before they are subjected to a fabric-forming operation, to the action of an aqueous emulsion having in disperse phase a water-insoluble organic swelling agent and substantially removing said agent from the materials before they are subjected to the action of any hot aqueous medium.

2. Process for increasing the tenacity and the extensibility of artificial filaments, threads, yarns and like materials containing organic derivatives of cellulose, which comprises stretching the materials while they are under the action of an aqueous emulsion having in disperse phase a water-insoluble organic swelling agent, permitting said materials, before they are subjected to a fabric-forming operation, to shrink while under the action of an aqueous emulsion having in disperse phase a water-insoluble organic swelling agent and substantially removing said agent from the materials before they are subjected to the action of any hot aqueous medium.

3. Process for increasing the extensibility of artificial filaments, threads, yarns and like materials containing organic derivatives of cellulose, which have been stretched to increase their tenacity, which comprises subjecting the materials, before they are subjected to a fabric-forming operation and in the absence of tension sufficient to stretch them, to treatment with an aqueous emulsion having in disperse phase a water-insoluble organic swelling agent and substantially removing said agent from the materials before they are subjected to the action of any hot aqueous medium.

4. Process for increasing the extensibility of artificial filaments, threads, yarns and like materials containing cellulose acetate, which have been stretched to increase their tenacity, which comprises subjecting the materials, before they are subjected to a fabric-forming operation and in the absence of tension sufficient to stretch them, to treatment with an aqueous emulsion having in disperse phase a water-insoluble organic swelling agent and substantially removing said agent from the materials before they are subjected to the action of any hot aqueous medium.

5. Process for increasing the extensibility of artificial filaments, threads, yarns and like materials containing organic derivatives of cellulose, which have been stretched to increase their tenacity, which comprises subjecting the materials before they are subjected to a fabric-forming operation and in the absence of tension sufficient to stretch them, to treatment with an aqueous emulsion of which the disperse phase comprises a water-insoluble organic swelling agent and a water-insoluble diluent and substantially removing said agent from the materials before they

are subjected to the action of any hot aqueous medium.

6. Process for increasing the extensibility of artificial filaments, threads, yarns and like materials containing organic derivatives of cellulose, which have been stretched to increase their tenacity, which comprises subjecting the materials before they are subjected to a fabric-forming operation and in the absence of tension sufficient to stretch them, to treatment with an aqueous emulsion of which the disperse phase comprises at least about 50% of a water-insoluble organic swelling agent and substantially removing said agent from the materials before they are subjected to the action of any hot aqueous medium.

7. Process for increasing the extensibility of artificial filaments, threads, yarns and like materials containing organic derivatives of cellulose, which have been stretched to increase their tenacity, which comprises subjecting the materials, before they are subjected to a fabric-forming operation and in the absence of tension sufficient to stretch them, to treatment with an aqueous emulsion of which the disperse phase comprises at least about 50% of a water-insoluble organic swelling agent and constitutes at least about 10% of the emulsion and substantially removing said agent from the materials before they are subjected to the action of any hot aqueous medium.

8. Process for increasing the extensibility of artificial filaments, threads, yarns and like materials containing organic derivatives of cellulose, which have been stretched to increase their tenacity, which comprises subjecting the materials, before they are subjected to a fabric-forming operation and in the absence of tension sufficient to stretch them, to treatment with an aqueous emulsion of which the disperse phase comprises at least about 50% of a water-insoluble organic swelling agent and constitutes 30-50% of the emulsion and substantially removing said agent

from the materials before they are subjected to the action of any hot aqueous medium.

9. Process for increasing the extensibility of artificial filaments, threads, yarns and like materials containing organic derivatives of cellulose, which have been stretched to increase their tenacity, which comprises subjecting the materials, before they are subjected to a fabric-forming operation and in the absence of tension sufficient to stretch them, to treatment with an aqueous emulsion having in disperse phase a chlorinated hydrocarbon which is a latent solvent for the materials, and substantially removing said latent solvent from the materials before they are subjected to any hot aqueous medium.

10. Process for increasing the extensibility of artificial filaments, threads, yarns and like materials containing organic derivatives of cellulose, which have been stretched to increase their tenacity, which comprises subjecting the materials before they are subjected to a fabric-forming operation and in the absence of tension sufficient to stretch them, to treatment with an aqueous emulsion having in disperse phase a water-insoluble organic swelling agent, said emulsion being prepared with the aid of an emulsifying agent, and substantially removing said agent from the materials before they are subjected to the action of any hot aqueous medium.

11. Process for increasing the extensibility of artificial filaments, threads, yarns and like materials containing organic derivatives of cellulose, which comprises subjecting stretched materials, before they are subjected to a fabric-forming operation, to the action of an aqueous emulsion having in disperse phase a water-insoluble organic swelling agent, said emulsion being stabilized with the aid of a protective colloid, and substantially removing said agent from the materials before they are subjected to the action of any hot aqueous medium.

HENRY DREYFUS.